

Aug. 24, 1937.

F. M. DAMITZ

2,090,623

VARNISHED CAMBRIC

Original Filed April 11, 1934



*Fig. 3*



*Fig. 5*



INVENTOR.

*Frederick M. Damitz,*

BY

*George D. Richards*

ATTORNEY.



## UNITED STATES PATENT OFFICE

2,090,623

## VARNISHED CAMBRIC

Frederick M. Damitz, Irvington, N. J., assignor  
to Irvington Varnish & Insulator Co., Irving-  
ton, N. J., a corporation of New Jersey

Original application April 11, 1934, Serial No.  
720,150. Divided and this application Novem-  
ber 4, 1935, Serial No. 48,258

4 Claims. (Cl. 91—67.9)

This invention relates, generally, to varnished cambrics and the invention has reference, more particularly, to a novel improved varnished cambric for use as insulation for cables and for other purposes requiring a high quality insulating material, the said varnished cambric being designed for ready identification as to its source at any time. This application is a division of my co-pending application, Serial No. 720,150.

10 There has been a long felt need in the electrical cable business for a varnished cambric having means for readily identifying the source of the cambric or the cable manufacturer, and possessing high dielectric strength, high insulation resistance and a high dielectric constant, the said varnished cambric to have a low power factor, as well as possessing great water resistance, heat resistance and oil resistance.

The principal object of the present invention is 20 to provide a novel varnished cambric having the above recited desirable qualities, the varnish film of the cambric being translucent so that identifying indicia or other markings on the cambric are easily legible.

25 Another object of the present invention lies in the provision of a varnished cambric of the above character having a varnish film comprising translucent asphaltic material in combination with linseed and China-wood oils.

30 Other objects of this invention, not at this time more particularly enumerated, will be clearly understood from the following detailed description of the same.

Varnished cambrics as heretofore manufactured may be classified in two classes depending on their color, whether yellow or black. Yellow varnished cambrics are quite generally made by coating cambric with an all drying oil. In some rare instances small amounts of gums and resins are added to the drying oil, but such additions tend to make the varnish film brittle and hence are seldom used. The drying oil used in producing yellow varnished cambrics is generally a combination of China-wood oil and linseed oil and 45 when these oils dry out and oxidize the film formed goes through two phases.

During the first phase, i. e., when the varnish is changing from a liquid to a solid, it is absorbing oxygen without the elimination of any other products. If, after the varnish has completely saturated itself with oxygen, the reaction ceased, it would be an ideal condition, but such is not the case for as long as the oxidized film is in contact with the air it continues to react with oxygen by 55 taking on oxygen and splitting off radicals known

as substitution products. Among these substitution products are water, glycerine, acrolein, aldehydes, non-volatile acids, and volatile fatty acids, which latter are further sub-divided into the water soluble and insoluble fatty acids. The water soluble fatty acids are electrolytic and therefore conductors, and hence lower the electrical resisting properties of the varnished cambric.

Furthermore, the decomposition which the film goes through results in the production of a porous structure which becomes capable of absorbing a large proportion of moisture and at the same time the film becomes brittle. Thus, the yellow varnish film is entirely of an oxidizing nature and is continually tending to disintegrate. Although the yellow varnish film is translucent and hence can be seen through for reading identifying indicia on the cambric, yet, owing to the rapid deterioration of this film and to its relatively poor insulating qualities, the same does not rate as a high grade insulating material.

Black varnished cambrics are made by coating cambric with an insulating varnish composed of inert black non-oxidizing asphalts and pitches in combination with drying oils. The asphalts and pitches are decidedly better insulators or dielectrics than the yellow gums and resins or the drying oils themselves. The varnish films or coatings of these black varnished cambrics are black and opaque, however, so it is impossible for identifying indicia on the cambric to be seen through the film. Furthermore, attempts to print or otherwise mark identifying indicia on the outer surface of the varnished film of the cambric have met with failure because of the ease with which such markings or indicia rub off in use.

The method of marking and varnishing my varnished cambric is clearly illustrated in the accompanying drawings, in which:

Fig. 1 is a schematic view of a plant used for producing the varnished cambric of this invention.

Fig. 2 is an enlarged sectional view taken along line 2—2 of Fig. 1.

Fig. 3 is an enlarged fragmentary plan view of the printed cambric.

Fig. 4 is an enlarged view taken along line 4—4 of Fig. 1.

Fig. 5 is an enlarged fragmentary plan view of the finished varnished cambric, and

Fig. 6 is an enlarged sectional view taken along line 6—6 of Fig. 1.

Similar characters of reference are employed in said views, to indicate corresponding parts.

In carrying out my invention, I print, stencil or otherwise mark the cambric or base cloth with suitable identifying characters, such as the trade-mark of the cable manufacturer or that of the varnished cambric manufacturer and then coat the printed cambric with the novel varnish of this invention. In preparing this varnish I use transparent or translucent material such as intermediate grades of cottonseed oil pitch having a viscosity range of from 10 to 30 degrees MacMicheal, i. e. when employing MacMicheal viscometer and using a No. 27 wire and a two centimeter bob at 25° C., the cottonseed pitch having been thinned somewhat with a mineral spirit such as "Varnolene". If desired, instead of using cottonseed oil pitch I may use linseed oil pitch, fish oil pitch, wool wax pitch, wool oil pitch, decolorized pitches such as those bleached with sulphur chloride, and various cashew shell oil combinations. These pitches when cooked with oils into varnishes, produce a finished translucent or substantially transparent product varying in color from a dark yellow to a deep brown and in some instances to a reddish brown.

As an example of the novel varnish employed in the present invention, the following ingredients are used in the percentages given by weight:

|                                                                  | Percent<br>by<br>weight |
|------------------------------------------------------------------|-------------------------|
| Cotton oil pitch (viscosity range of from 10° to 30° MacMicheal) | 17.6                    |
| Linseed oil                                                      | 4.0                     |
| China-wood oil                                                   | 19.4                    |
| Litharge                                                         | .5                      |
| Manganese resinate                                               | 1.2                     |
| Mineral spirit ("Varnolene")                                     | 57.3                    |

In producing the varnish I mix 200 lbs. cottonseed oil pitch (60% solid and 40% mineral spirit, viscosity range from 10° to 30° MacMicheal, i. e. by MacMicheal viscometer using a No. 27 wire and a two centimeter bob at 25° C.) with 6 gallons of linseed oil and heat the mixture to approximately 600° F. This hot mixture is kept at 600° F. for from one to two hours during which period polymerization and some oxidation takes place, thereby increasing the viscosity of the mixture and giving the same the desired body. During this heating period, the mixture may be blown with either air, nitrogen or carbon dioxide thereby hastening polymerization, although such blowing is not necessary.

Six pounds of litharge serving as a drier is then added and mixed thoroughly into the hot pitch-oil mixture. Twenty gallons of China-wood oil is also added with stirring. The cold China-wood oil will cause the temperature of the pitch-oil-litharge mixture to drop considerably so the mixture is then heated somewhat to bring its temperature up to approximately 540° F., after which the mixture is chilled by adding thereto 8 more gallons of China-wood oil and then held for body at 450° F., after which 14 lbs. of manganese resinate serving as a drier is stirred into the mixture. The varnish base thus formed is allowed to cool somewhat and when at a temperature of from 300° to 350° F. the same is thinned with 100 gallons of "Varnolene" (a petroleum hydrocarbon or mineral spirit having a distillation range of 310° to 420° F.). The novel varnish is now complete and is of brownish color and when applied in the form of a film and allowed to dry the same forms a smooth, flex-

ible, durable and substantially transparent coating.

In producing the varnished cambric of this invention, a web 1 (see Figs. 1 and 2) of cambric fed from a roll 2 is passed over a printing roll 3 that is supplied with ink as by an inking roll 4. The printing roll 3 serves to print the desired indicia 10 such as a trade name or manufacturer's name on the web 1 which web may be a plain cambric, a colored cloth, or a fabric provided with a design or designs thereon. The thusly printed fabric is shown in Figs. 3 and 4.

After leaving the printing roll 3, the web 1 is passed through the novel varnish 5 of this invention which varnish is contained in a pan 6 mounted in a vertical heating tower 7. If desired, the varnish may be further thinned by use of "Varnolene" or any other mineral spirit such as naphtha, benzene, toluol, benzol, xylol and high flash naphtha before passing the web 1 therethrough. After emerging from the varnish 5, the web passes upwardly within the vertical heating tower 7, the air within which is maintained at a temperature of from 280° to 230° F. as by heating coils 8. The web is shown passing over a roll 12 at the top of tower 7 and then downwardly through more varnish 5 contained within a second pan 6'. From the pan the web passes upwardly and over a roll 13 at the top of the tower and then downwardly and out of the tower. Within the tower 7 the solvent is driven off of the varnished cambric and the varnish is oxidized and polymerized. After leaving the tower 7, the varnished web 1, having the varnished film or coating 11 on its outer surface, is rolled on a roll 9.

Although in Fig. 1, I have shown the web as dipped but twice, ordinarily the web would be dipped three, four or even more times to build up the desired thickness of film 11, and after each dip the web is dried within the heating tower. Thus, for a 12 mill finished product, using a 4½ mill cloth, the web will be dipped four times, having the varnish at about 30° Baumé for the first coat and 35° Baumé for the subsequent coats, using "Varnolene" as a solvent for thinning. If desired, instead of dipping the fabric, the varnish may be sprayed, brushed or roller coated thereon.

The varnished cambric thus produced has exceptionally high insulating qualities and the translucent or substantially transparent film or coating 11 enables the indicia 10 to be readily legible as illustrated in Fig. 5. Tests show that the dielectric strength of this novel varnished cambric to be 20 to 30% higher than yellow varnished cambrics and the insulation resistance at room temperature is 10<sup>3</sup> or substantially one thousand times as great as that of yellow varnished cambrics. At 100° C. the insulation resistance is 10<sup>6</sup> times that of the yellow. The dielectric constant of this novel varnished cambric is approximately 4 as compared to 5½ to 6 for yellow varnished cambric. At room temperature, the power factor of my varnished cambric is of the magnitude of about 3½ % as compared to 10 to 12% for yellow varnished cambric. At 60° C. the power factor of my varnished cambric is of the magnitude of 4 to 5% as compared with 30% for yellow varnished cambric, while at 80° C. the power factor of my cambric is 5 to 7% as compared to 70 to 90% for yellow varnished cambric. My varnished cambric also shows superiority over yellow varnished cambric as to water and heat resistance. After 24 hrs. of

Immersion in water the yellow varnished cambric will have absorbed 12 to 15% of its volume of water and its dielectric strength will be reduced about 60%, whereas my cambric after a like im-

5 mersion will absorb but 4 to 5% of its volume of water and its dielectric reduced but 30 to 40%.

Black varnished cambrics as heretofore produced have higher insulating properties than the yellow varnished cambrics, but since these 10 black varnished cambrics have opaque films they are not suitable for my purpose where a substantially transparent film is desired in order to read indicia on the web or cambric and hence I have made no comparison between the insulating 15 properties of black varnished cambrics and my varnished cambric.

The cottonseed oil pitch ingredient of my varnish composition serves to stabilize the linseed oil and the China-wood oil and effectively 20 prevents these ingredients from excessive oxidation. It appears that the pitch serves as a matrix for surrounding the oxidizing oils, i. e. linseed and China-wood oil, so that these oils do not come into contact with sufficient oxygen to produce 25 excessive oxidation.

It will be understood that some variation may be made in the relative percentage of the several ingredients of my varnish composition while still retaining the high insulating qualities of the 30 same and the same transparency or translucency whereby the indicia 10 may be read. The percentages of the oils should not be unduly increased, however, because they will then decrease the electrical resisting properties of the varnish 35 and render it less moisture proof. Too much pitch on the other hand will decrease the flexibility of the film and will lower its resistance to oil solubility (i. e. transformer oil for example).

If desired, instead of using cottonseed oil pitch 40 I may use linseed oil pitch, fish oil pitch, wool wax pitch, wool oil pitch, decolorized pitches such as those bleached with sulphur chloride and cashew shell oil combinations. These pitches should be thinned, if necessary, so as to have 45 substantially the same viscosity range as that of the cottonseed oil pitch.

It is to be understood that I may use quantities of other oils partly in lieu of or in addition to the linseed oil and China-wood oil in my varnish.

For example, I may add quantities of the following oils, namely perilla oil, soya bean oil, cottonseed oil, rapeseed oil, fish oil, paraffin oils and higher grease oils.

As many changes could be made in the above 5 construction and many apparently widely different embodiments of this invention could be made without departing from the scope thereof, as defined by the following claims, it is intended that all matter contained in the above description 10 or shown in the accompanying drawings shall be interpreted as illustrative and not in a limiting sense.

I claim:—

1. A varnished cambric comprising, a base 15 cloth having indicia marked thereon and a substantially transparent varnish overlying said base cloth and said indicia, whereby said indicia may be seen through said varnish, said varnish constituting a combination of a drying oil and a 20 substantially transparent vegetable oil pitch, said varnish having high insulating efficiency.

2. A varnished cambric comprising, a base 25 cloth having indicia marked thereon and a substantially transparent varnish overlying said base cloth and said indicia, whereby said indicia may be seen through said varnish, said varnish comprising a drying animal oil and a substantially transparent pitch, said pitch serving as a matrix for the drying oil.

3. A varnished cambric comprising, a base 30 cloth having indicia marked thereon and a substantially transparent varnish overlying said base cloth and said indicia, whereby said indicia may be seen through said varnish, said varnish comprising a mixture of linseed oil and China-wood oil as a drying oil and substantially transparent cottonseed oil pitch, said pitch serving as a matrix for the drying oil.

4. In a varnished cambric having a base cloth 40 provided with markings thereon, a substantially transparent varnish film overlying said base cloth and said indicia, said varnish film comprising a mixture of linseed oil and China-wood oil as a drying oil and a substantially transparent cottonseed oil pitch having a viscosity 45 range of from 10 to 30 percent MacMicheal and serving as a matrix for the drying oil.

FREDERICK M. DAMITZ.